

## UNITED STATES PATENT OFFICE

2,456,567

## AMINOTRIAZINE PRODUCT

Milton J. Scott, Springfield, Mass., assignor to  
 Monsanto Chemical Company, St. Louis, Mo., a  
 corporation of Delaware

No Drawing. Application September 1, 1944,  
 Serial No. 552,381

6 Claims. (Cl. 260—67.6)

1

This invention relates to the preparation of water-insoluble metal salts of ammeline-aldehyde reaction products and to fibrous materials having such products deposited thereon.

An object of this invention is to provide water-insoluble metal salts of ammeline-aldehyde reaction products. A particular object of this invention is to provide fibrous material having associated therewith water-insoluble metal salts of ammeline-aldehyde reaction products.

These and other objects are attained according to this invention which comprises forming an aqueous solution of a reaction product of ammeline and an aldehyde, said aldehyde having a solubility in water of at least three parts for every one hundred parts of water at 20° C. then precipitating said reaction product by the addition of a water-soluble compound of a metal selected from the group consisting of the heavy metals and the metals of group 2A of the periodic system.

According to one embodiment of this invention, fibrous materials are treated with aqueous alkaline solutions of the ammeline-aldehyde reaction products described above and a water-soluble compound of a heavy metal or of a metal of group 2A of the periodic system is added to the treated fibrous material, thereby precipitating the metal salt of the ammeline-aldehyde reaction product on the fibrous material. Thereafter, the ammeline-aldehyde product may be polymerized by heating, either before, during or after removal of the aqueous medium.

According to a further embodiment of this invention, webs or sheets of fibrous materials such as paper or textiles may be impregnated with the water-soluble ammeline-aldehyde reaction product, a metal compound of the type described above incorporated in the web and the resulting product heated to dry the web or sheet, and/or polymerize the precipitated salt of the ammeline-aldehyde reaction product.

Other methods of incorporating the insoluble salts of this invention on fibrous materials include treating the fibrous materials with an aqueous slurry or emulsion of the insoluble salt or treating the fibrous material with the precipitating metal compound and thereafter incorporating the water-soluble ammeline-aldehyde condensation product.

For convenience, the reaction product of ammeline and formaldehyde is used to illustrate the invention in the following examples, but it is to be understood that the invention is not so limited. Where parts are mentioned, they are parts by weight.

2

## Example I

A mixture of 127 parts (1 mol) of ammeline, 243 parts (3 mols) of an aqueous solution of formaldehyde (37% HCHO) and sufficient sodium hydroxide (in a 5% aqueous solution) to produce a pH of about 9.3 (glass electrode), is boiled under reflux conditions at atmospheric pressure for about 30 minutes and then cooled to room temperature. The product comprises an aqueous solution of the sodium salt of trimethylol ammeline. Addition of 158 parts of alum ( $KAl(SO_4)_2 \cdot 12H_2O$ ) to this solution, preferably with stirring, results in the formation of a white flocculent precipitate which may be recovered by filtration and drying at a low temperature e. g. 50–70° C. The solid, water-insoluble product comprises the aluminum salt of trimethylol ammeline.

## Example II

Example I is repeated except that in place of the alum employed in Example I, an equivalent amount of calcium chloride hexahydrate (110 parts) is employed. The product comprises the calcium salt of trimethylol ammeline.

## Example III

A mixture of 127 parts (1 mol) of ammeline, 243 parts (3 mols) of aqueous formaldehyde solution (37% HCHO) and sufficient sodium hydroxide (in a 5% aqueous solution) to produce a pH of about 9.3 (glass electrode), is boiled under reflux conditions for about 100 minutes at atmospheric pressure. After cooling 79 parts of alum ( $KAl(SO_4)_2 \cdot 12H_2O$ ) is added and causes a white flocculent precipitate to form. The precipitated product comprises the aluminum salt of a partial polymer of trimethylol ammeline.

## Example IV

A mixture of 127 parts (1 mol) of ammeline, 162 parts (2 mol) of an aqueous formaldehyde solution (37% HCHO) and sufficient sodium hydroxide (in a 5% aqueous solution) to produce a pH of about 9.3 (glass electrode) is boiled under reflux conditions for about 30 minutes at atmospheric pressure. After cooling, 158 parts of alum ( $KAl(SO_4)_2 \cdot 12H_2O$ ) are added whereby a white flocculent precipitate comprising the aluminum salt of dimethylol ammeline is formed.

Numerous variations may be introduced into the process of forming the insoluble salts of this invention. Thus, water-soluble ammeline-aldehyde reaction products may be precipitated while still substantially unpolymerized and, when desired, the precipitated product thereafter poly-

merized by heating, or the water-soluble products may be partially polymerized prior to precipitation and, when desired, the polymerization continued after the formation of the water-insoluble metal salts. However, it is preferred that prior to the addition of the precipitating compound, the ammeline-aldehyde reaction product not be polymerized beyond the state of solubility in aqueous alkaline solutions.

In preparing the ammeline-aldehyde condensation or reaction products, the proportions of ammeline and aldehyde may be substantially varied. Thus, molar ratios of combined aldehyde per mol of ammeline may vary from 1:1 to 4:1, and higher ratios of aldehyde to ammeline may be present in the reaction mixture. Furthermore, the pH of the reaction mixture may be substantially varied. Generally, it is preferred that sufficient alkaline material be present so that the reaction mixture has a pH of 7 or higher and preferably a pH in the range 8.0-9.5 (glass electrode) and especially about 9-9.3.

The aldehydes employed in making the water-soluble ammeline-aldehyde condensation product are characterized by having a solubility in water of at least three parts for every 100 parts of water at 20° C. Examples of such aldehydes are the lower aliphatic aldehydes, for example, formaldehyde, acetaldehyde, propionaldehyde, butyraldehyde, as well as aldehydes substituted by hydrophilic groups, as for example, such hydroxy aldehydes as glycolic aldehyde, glyoxylic aldehyde; unsaturated aldehydes such as croton-aldehyde, acrolein, tiglaldehyde; halogen substituted aldehydes such as, chloral; dialdehydes such as glyoxal.

The alkaline reagents used in making the water-soluble ammeline-aldehyde reaction products comprise the basic reacting compounds of the metals of group 1A of the periodic system as for example, the hydroxides and carbonates of lithium, sodium, and potassium, ammonium hydroxide, ammonium carbonate, quaternary ammonium bases such as dimethyl dibenzyl ammonium hydroxide, trimethyl benzyl ammonium hydroxide, tetraethyl ammonium hydroxide, tetraethanol ammonium hydroxide and the like.

In place of the alum and calcium chloride employed in the above examples, other water soluble compounds of metals from the group consisting of aluminum, magnesium, the heavy metals and the metals of group 2A of the periodic system may be used. Thus, for example, the water-soluble nitrates, chlorides, hydroxides of aluminum, calcium, barium, strontium, zinc, cadmium, copper, silver, iron, cobalt, nickel, chromium, magnesium and the like may be used.

The insoluble metal salts of this invention may be used for various purposes, for example, as molding compounds, resinous bases for coating or impregnating compositions and the like. During or after the application of these metal salts they may be polymerized under heat or under heat and pressure to provide insoluble, infusible products.

The following are examples illustrating the use of the metal salts of this invention, particularly for incorporation with fibrous materials.

#### Example V

8 parts of a 12% solution of sodium trimethylol 70 ammeline prepared as shown in Example I, are added to a beater or hollander containing 1350 parts of a 2% Northern Kraft beater pulp stock having a pH of about 9 and a freeness of 12 seconds (as determined with a standard Williams 75

freeness tester with 2.5 grams of the beater slurry at 25° C. and 0.25% consistency). After thorough mixing in the beater the slurry is diluted to about 21,000 parts with water and 0.07 part of alum ( $KAl(SO_4)_2 \cdot 12H_2O$ ) added to precipitate the sodium trimethylol ammeline onto the pulp fibers. Paper sheets are felted out from the resulting slurry by the Technical Association of the Pulp and Paper Industry Standard Method #T205. The sheets are heated for 10 minutes under low pressure e. g. 25 pounds per square inch at 110° C. and then for 30 minutes at 150° C. to remove the water and polymerize the aluminum trimethylol ammeline.

15 An excess of alum or other precipitant may be used in obtaining the products of this invention wherever it is advantageous as in the paper industry where alum is used to control the pH of the beater slurry and to modify the properties of the paper.

20 Paper sheets made as described above are found to possess increased strength, particularly increased wet strength as compared with paper made by felting untreated fibers of the same pulp slurry.

25 In a similar manner other insoluble metal salts of ammeline-aldehyde reaction products may be incorporated in paper by precipitating the salts in the beater stock prior to felting out the paper sheet. Thus, paper containing the insoluble salts 30 described in Examples II, III, and IV may be prepared in the manner set forth in Example V to produce paper having characteristics similar to those of the product described in Example V.

35 The process of preparing paper having incorporated therein insoluble metal salts of ammeline-aldehyde reaction products as set forth in Example V may be substantially varied. For example, the process is not limited to the particular pulp stock used in Example V and other fibers, concentrations of fiber and stock having other freeness values may be used.

40 The amount and concentration of the soluble ammeline-aldehyde product that is introduced 45 may be substantially varied. However, since only a limited amount of the insoluble salt is adsorbed by the fibers there is generally no advantage in greatly exceeding the amount that can be adsorbed. Thus, while there may be some variation due to the particular conditions existing in the beater stock, e. g. degree of freeness, degree of dilution, type of fiber, etc., in general, from about 1 to 5 parts of the soluble ammeline-aldehyde product is incorporated in the beater stock for every 100 parts of fiber.

50 The amount of the precipitating metal compound that is incorporated in the beater is generally such that one chemical equivalent of the metal compound is incorporated per chemical equivalent of ammeline residue in the ammeline-aldehyde product i. e. in the case of the alum used above, one mol is employed for three mols of the ammeline residue present in the ammeline-aldehyde product. However, a lesser amount of the metal compound may be used, when desired, and particularly when the soluble ammeline-aldehyde product is partially polymerized prior to precipitation and as pointed out above, a larger amount may be desirable, e. g. to affect the pH of the stock and to modify the characteristics of the product.

55 The fibrous materials which may be treated with the water-insoluble salts of this invention include cellulose fibers such as, for example, wood pulp or cotton rag fibers used in paper making; natural fibers such as, for example, silk,

wool, cotton, flax, hemp, jute, etc., used in textile manufacture and synthetic fibers such as, for example, regenerated cellulose, rayons, cellulose acetate, vinyl chloride-vinyl acetate copolymers, vinyl chloride-methyl acrylate copolymers and polyamide fibers.

The following is an example of a molding composition made from the products of this invention.

*Example VI*

100 parts of the precipitated, dried product described in Example I are formed into a molding composition by admixture with 100 parts of wood flour and 2 parts of aluminum stearate as a lubricant, in the usual manner for preparing single-stage molding compositions, i. e. by admixing the ingredients and then advancing the polymerization of the resin as desired on hot milling rolls. The product is molded in a cup-shaped mold at 2,000-4,000 pounds per square inch and 140-170° C. for 2 minutes to form a molded product having a high degree of toughness and water resistance.

In place of the product of Example I, other insoluble metal salts of ammeline-aldehyde products may be used, e. g. the products described in Examples II, III and IV or their partially polymerized products. Other fillers or mixtures thereof may be employed in place of wood flour, e. g., mica, quartz, asbestos, etc. Other lubricants may be used, e. g., calcium stearate or for certain purposes the lubricant may be omitted entirely. The proportion of filler may be substantially varied but generally from 40 to 60 parts of filler are employed for every 60 to 40 parts of the ammeline-aldehyde metal salt when molded products containing fillers are desired.

A particular advantage of the process of this invention comprises the use of water-soluble substantially unpolymerized material which may be converted into the water-insoluble state without resort to heating and like polymerization conditions. Such a process leads to unexpected results, not obtainable with materials requiring a polymerization step in the process of converting the products to a water-insoluble state.

Furthermore the insoluble salts of ammeline-aldehyde condensation products may be reconverted into the soluble state by chemical means e. g. by treatment with a solution of sodium hydroxide or other hydroxides of the alkali metals. Thus, a particular advantage of the present invention as exemplified by the use of the products of this invention in treating paper, resides in the ability to rework the treated paper. Thus, the "broke" may be treated with alkali such as the hydroxides of the metals of group IA of the periodic system whereby the ammeline-aldehyde products are dissolved. The fibrous material

may then be freed from the resulting slurry or the slurry may be again processed preferably in admixture with fresh materials as set forth hereinbefore whereby the ammeline-aldehyde product is again precipitated on the fibers.

It is understood that the above description is given by way of illustration only, and not of limitation, and that deviations are possible within the spirit of the invention.

What is claimed is:

1. A process which comprises adding a water-soluble compound of a metal selected from the group consisting of aluminum, magnesium, the heavy metals and the metals of group 2A of the periodic system, to the product obtained by reacting at a pH of 8-9.5 ammeline and an aqueous solution of an aldehyde having a solubility in water of at least 3 parts for each 100 parts of water at 20° C., whereby said reaction product of ammeline and said aldehyde is precipitated, the ammeline being reacted with the aldehyde to an extent which is insufficient to cause the ammeline-aldehyde reaction product to precipitate from the aqueous alkaline medium prior to addition of the metal compound and the amount of the metal compound being sufficient to provide a chemical equivalent of the metal for each molecule of ammeline.
2. A process as defined in claim 1 in which the aldehyde is formaldehyde.
3. A process as defined in claim 1 in which the water-soluble metal compound is alum.
4. A process as defined in claim 1 in which the aldehyde is formaldehyde and the water-soluble metal compound is alum.
5. A process as defined in claim 1 in which the metal compound is a calcium compound.
6. A process as defined in claim 1 in which the aldehyde is formaldehyde and the metal compound is a calcium compound.

MILTON J. SCOTT.

REFERENCES CITED

The following references are of record in the file of this patent:

UNITED STATES PATENTS

| Number    | Name        | Date          |
|-----------|-------------|---------------|
| 2,191,362 | Widmer      | Feb. 20, 1940 |
| 2,208,653 | Whitehead   | July 23, 1940 |
| 2,217,667 | Bruson      | Oct. 15, 1940 |
| 2,291,080 | Hofferbert  | July 28, 1942 |
| 2,318,121 | Widmer      | May 4, 1943   |
| 2,321,451 | Bauer       | June 8, 1943  |
| 2,356,719 | Wohnsiedler | Aug. 22, 1944 |
| 2,364,726 | Landolt     | Dec. 12, 1944 |
| 2,377,868 | D'Alelio    | June 12, 1945 |